

Nov. 14, 1933.

O. A. TOWNSEND

1,934,779

COLOR PHOTOGRAPHY

Filed April 30, 1932



INVENTOR.  
O. A. Townsend  
BY *Mark H. Clark*  
ATTORNEYS.

## UNITED STATES PATENT OFFICE

1,934,779

## COLOR PHOTOGRAPHY

Oliver Arnold Townsend, Berhampore, Wellington, New Zealand, assignor to Tru Colour Film Limited, Wellington, New Zealand

Application April 30, 1932, Serial No. 608,567, and in New Zealand June 5, 1931

4 Claims. (Cl. 95—2)

This invention relates to photography, and more particularly to the production of films for producing natural color pictures.

The object of the invention is to provide an improved process by the use of which there can be produced colored positive film wherein colors are reproduced more naturally and with less exaggeration or artificialness than in positive films produced by known processes, and also wherein a plurality of colored images can be printed in a single emulsion common to standard commercial films, so that the colors are non-fugitive or are rendered practically indestructible with ordinary usage.

15 The process is simple and can be carried out in any well equipped cine or other photographic laboratory, by means of known apparatus, so as to produce positive film containing or having incorporated therein an increased variety of 20 natural color tones, with the images sharply and clearly defined, avoiding fringe or fuzziness, and in the case of a film used for picture projection, without flicker and undue loss of light in the projected picture.

25 The invention consists, briefly, in producing positive film by printing a positive image in one side of the emulsion of a single emulsion film from a negative image formed by a combination of colored light rays; developing said positive 30 image, subjecting the latter to color toning treatment, followed by controlled fixation treatment; re-converting the untoned portion of the printed image to a condition in which it will take further printing; printing through the reverse side of 35 the emulsion into said reconverted portion of the first printed image and unprinted portion of the emulsion, a second positive image from a negative image formed by a different combination of light rays; developing and fixing said second positive 40 image and color toning same so that the two colored positive images combine to reproduce varying color effects.

The invention further consists in printing the first positive image, above referred to, in the 45 outer side of the emulsion, the second positive image being printed in the emulsion through the support therefor, which order of procedure, together with the color toning of the first positive image, and controlled fixation of said color 50 toning to provide an untoned portion, followed by the conversion and utilization of the untoned portion of the first positive image in the production of the second positive image, with development of the latter and said untoned color 55 toned portion, and a further color toning of the

aforesaid untoned portion when color toning the second positive image, results in there being obtained in the finished positive film such an intimate mixture or intermingling of colors, that tones and color shades not obtainable with known two color processes, are enabled to be reproduced photographically.

In order that the invention may be better understood, it will now be described in detail, the following being a practical working description of the process.

The one figure of the attached drawing diagrammatically illustrates my invention more elaborately described in the following description:

70 Standard single emulsion film is used in the formation of the positive, the latter being printed from a negative film or films the images on which have been obtained with or without the aid of separate, or combined red and yellow or orange, 75 and blue or blue green filters, screens, or color selectors, in any known manner, by the use of any suitable cameras.

In order to produce the positive film, a positive image of suitable weight is printed in the outer 80 side of the emulsion of the film from a negative image formed by red orange yellow green light rays, to produce an image representing the blue green portion and developed by means of a suitable developer, a developer consisting of sodium 85 sulphite, potassium metabisulphite, diamidophenol hydrochloride and water, being found to give good results in this connection.

Following the development of the positive image just printed, the film is washed for approximately 90 five minutes, and toned blue in a bath consisting of ferric chloride, oxalic acid, nitric acid, potassium ferricyanide, and water, said ingredients being used in the following proportions:—ferric chloride 36 grains to 72 grains, but preferably 48 95 grains; oxalic acid 6 grains to 20 grains, but preferably 12½ grains; nitric acid approximately 180 minims; potassium ferricyanide 48 grains to 96 grains, but preferably 60 grains, and water approximately 240 fluid ounces.

100 The treatment of the film in this last mentioned toning bath, results in the blue tone being absorbed or deposited only in that portion of the positive image in the outer layer or portion of the emulsion, so that when the depth of the image varies or is irregular, shallow portions or the half tones of said image, are fully toned or colored, while portions of the image of greater depth than said shallow portions or half tones, are not toned 105 110

or colored for their full depth, the remaining or unblued reduced silver of said deeper portions or shadows being converted to silver ferrocyanide.

The film is then rinsed, and after rinsing is treated in a bath consisting of sodium thiosulphate  $1\frac{3}{4}$  ounces to 8 ounces, but preferably 2 ounces  $3\frac{1}{2}$  grains; potassium metabisulphite  $\frac{1}{2}$  ounce to 2 ounces, but preferably  $\frac{3}{4}$  ounce  $3\frac{1}{2}$  grains; and water approximately 240 fluid ounces, which dissolves out the silver ferrocyanide from the blue toned portion of the image and secures fixation thereof, the fixation being controlled by time and temperature so as to leave an unfixed blue toned portion below the fixed blue portion, while the silver ferrocyanide in the deeper portions of the image is not toned blue, together with more or less, or some of the remaining silver bromide, is converted to insoluble silver thiosulphate. The fixation of the upper or outer layer of the blued portion of the image by the last described treatment prevents any re-development of said layer during further treatment of the film, and so gives where there is no underlay of red or yellow, the necessary blue where required film is now rinsed in water.

To print on the other side of the film and in order to enable the positive film therein to satisfactorily receive a print from the negative image formed by the violet blue green yellow light rays, that part of the emulsion not now consisting of silver bromide, excepting the fixed blued portion of the image, is converted to silver bromide, this being effected by immersion of the latter in a bath of ammonium carbonate  $\frac{1}{2}$  ounce to 2 ounces, but preferably  $\frac{3}{4}$  ounce; ammonium bromide  $\frac{1}{8}$  ounce to  $\frac{1}{2}$  ounce, but preferably  $\frac{1}{4}$  ounce, or the equivalent amount of bromine as a salt of this halogen; and water approximately 240 fluid ounces, which bath also has the effect of clearing out any blue stain remaining in the emulsion. That part or parts of the emulsion which does consist of silver bromide at the time of the reconversion operation is or are more or less re-sensitized during the latter, such re-sensitizing facilitating the obtaining of a fine grained second positive image, in the reverse side of the emulsion.

In preparing the bath last referred to it is advisable to first dissolve the ammonium carbonate in the water which has been boiled for the purpose, and allow the solution to cool before adding the ammonium bromide.

The film is then rinsed and dried in a suitable light, and the second positive image obtained by printing from the negative image formed by the violet blue green yellow light rays, into the converted silver bromide portion of the first positive image and the remaining silver bromide of the emulsion, the printing being done through the emulsion support. The last mentioned or second positive image is then developed by means of a suitable developer, fixed in a hypo bath, washed, and toned in a yellow red bath of uranium nitrate  $\frac{1}{4}$  ounce to  $\frac{1}{2}$  ounce, but preferably  $\frac{1}{4}$  ounce 50 grains; oxalic acid 60 grains to 100 grains, but preferably 80 grains; nitric acid approximately  $1\frac{1}{2}$  ounces; potassium ferricyanide 55 grains to 95 grains, but preferably 75 grains; and water approximately 160 fluid ounces.

Unless otherwise specified, proportions of ingredients are by avoirdupois system of weights.

The positive film is then fixed in a hypo bath, to reduce graininess and brighten the whole picture, and can be given such treatment in an appropriate bath or baths as may be desirable for

the purpose of intensifying any particular color or colors.

What I do claim and desire to obtain by Letters Patent of the United States of America is:—

1. A process for use in the production of photographic film with registering differently colored positive images thereon, consisting in printing an image in the outer side of the emulsion of a single emulsion film from a negative image formed by red, orange, yellow, green light rays; developing said image; subjecting the latter to treatment in a blue bath, whereby part of the image is blue toned, subjecting the partly blue toned image to controlled fixation to provide a fixed and an unfixed blue toned portions; reconverting the untoned portion of the image to silver bromide; printing a second positive image through the emulsion support into the reconverted portion of the first printed positive image and the unprinted silver bromide of the film, from a negative image formed by violet, blue, green, yellow light rays, developing and fixing said second positive image and color toning same and the unfixed color toned portion of the first image, in a yellow red bath.

2. The process of producing a photographic film having differently colored outer and inner superposed images therein which consists in printing and developing said images, but before fixing the film toning the outer image blue in a blue bath constituted to tone the outer image without affecting the inner image to the extent that the shallow or top portions of said outer image are completely toned whilst deeper portions of said outer image are not toned completely, converting the non-completely toned portions of the outer image into silver ferrocyanide, rinsing and fixing the entire film, toning the second image in a penetrating red yellow bath, rinsing the film and fixing the red yellow toned image.

3. The process of producing photographic film having differently colored positive images in opposite surfaces of a single emulsion which consists in printing an image from a negative formed by red orange yellow green light rays on the outer side of an emulsion, then developing said image, washing the film and toning the image blue to the extent that the shallow portions of said outer image are fully toned while portions of the image of greater depth are not completely toned, the remaining or deepest portions being converted to silver ferrocyanide, rinsing the film and treating the same in a bath containing sodium thiosulphate to dissolve out the iron silver ferrocyanide from the fully blue toned portion of the image and secure fixation thereof, but leaving an unfixed blue toned portion below the fixed blue portion while the silver ferrocyanide in the deepest portions of the outer image is not blue toned but is converted into insoluble silver thiosulphate, rinsing the film and treating the same in a bath containing ammonium bromide and ammonium carbonate to convert all the insoluble silver thiosulphate in the emulsion to light sensitive silver bromide, and printing on the opposite side of the emulsion an image from a negative formed by violet blue green yellow light rays.

4. A process as claimed in claim 2 in which the differently colored outer and inner superposed images are made on the same side of a common support.

OLIVER ARNOLD TOWNSEND.